

## UNITED STATES PATENT OFFICE

1,997,760

## VULCANIZATION OF RUBBER

Ira Williams, Woodstown, N. J., assignor to E. I. du Pont de Nemours & Company, Wilmington, Del., a corporation of Delaware

No Drawing. Application March 25, 1933,  
Serial No. 662,825

4 Claims. (Cl. 18—53)

This invention relates to the vulcanization of rubber and more particularly to a method whereby the acid deficiency of rubber may be corrected and the action of vulcanization accelerators facilitated.

It is well known that rubber which is deficient in fatty acid content produces a poor vulcanizate and that rubber from which all acidic material has been removed cannot be satisfactorily vulcanized. It is also known that many accelerators of vulcanization require the addition of considerable fatty acid in order to produce satisfactory acceleration. Accordingly, it has become a practice to add fatty acids of the higher fatty acid series to rubber mixes.

The fatty acids most commonly employed are stearic acid and oleic acid. The use of these and other high molecular weight fatty acids are disclosed in Patent 1,467,197, granted to W. F. Russell. While these acids will overcome the fatty acid deficiencies of rubber, they are objectionable in several respects. When employed in the presence of such accelerators as tetramethyl thiuram monosulfide or butyraldehyde-aniline condensation products, they have a retarding action on the vulcanization due to their acidity. When employed in amounts greater than about 1%, these materials bloom to the surface and destroy the tack of the unvulcanized rubber in such manner as to seriously interfere with fabricating operations.

An object of the present invention is to provide a class of materials which may be employed to correct the acid deficiency of rubber and at the same time to act as accelerator activators without exerting a retarding action on certain accelerators which are ordinarily deleteriously affected by fatty acids. A further object is to provide a class of acid supplying accelerator activators which are sufficiently soluble in rubber to permit them to be employed in the desired amounts without blooming to the surface. Still further objects are to improve the properties of rubber and to provide methods for effecting such improvement. Other objects are to provide new compositions of matter and to advance the art. Other objects will appear hereinafter.

These objects may be accomplished in accordance with my invention which comprises adding to a rubber mix, prior to vulcanization, certain

mono-carboxylic aliphatic acids, or their salts and thereafter vulcanizing. The mono-carboxylic acids and their salts which are to be employed in accordance with my invention comprise compounds of the type:



in which M represents hydrogen or an equivalent of a metal selected from the group comprising lead, mercury, cadmium and zinc and R represents a saturated or unsaturated alkyl group of more than one and less than 10 carbon atoms and in which the longest carbon chain is not more than 7 carbon atoms in length, or R may represent a saturated cyclic hydrocarbon group.

Among the acids which have been found to be particularly satisfactory for my purpose are propionic, butyric, isobutyric, crotonic, valeric, caproic, heptoic, ethyl propylacetic, 3-methyl-5-ethyl-hexoic, and hexahydrobenzoic acids, and their salts of lead, mercury, cadmium and zinc.

These acids are preferably employed by first forming the zinc salt and adding such salt to the rubber mix. However, if desired, these acids may be introduced into the rubber in the form of the free acid together with excess of the metallic oxide whereupon the metallic salt will be formed in the rubber. The use of the acid in the form of its salts will generally be preferred to avoid disadvantages attendant upon adding a material which may be volatile and of disagreeable odor.

In order to determine the effectiveness of this class of materials, a rubber mix was prepared having the following composition:

|                        | Parts by weight |
|------------------------|-----------------|
| Rubber                 | 100             |
| Carbon black           | 25              |
| Zinc oxide             | 5 40            |
| Sulfur                 | 3               |
| Mercaptobenzo-thiazole | .5              |

Various activating ingredients were added to this mix in the proportion of 3 parts of activating material to each 100 parts of rubber. The resulting mixes were then vulcanized at 287° F. for periods of 20, 30, 45 and 60 minutes, after which the tensile strengths at break in pounds per square inch were determined. The results of 50

some of these tests are shown in the following table: compounds in the class may be employed with satisfactory results, the proportions may be varied

*Tensile strength at break*

| Minutes<br>cure | Activator added |                      |                       |                    |                  |                       |                    |                       |                 |
|-----------------|-----------------|----------------------|-----------------------|--------------------|------------------|-----------------------|--------------------|-----------------------|-----------------|
|                 | None            | Zinc pro-<br>pionate | Zinc iso-<br>butyrate | Zinc hep-<br>toate | Crotonic<br>acid | Cadmium<br>propionate | Lead buty-<br>rate | Mercurous<br>caproate | Caproic<br>acid |
| 10              |                 |                      |                       |                    |                  |                       |                    |                       |                 |
| 20              | 1900            | 3000                 | 2630                  | 2675               | 3025             | 2850                  | 4550               | 4200                  | 3000            |
| 30              | 1375            | 3300                 | 2850                  | 3625               | 3675             | 2850                  | 4425               | 4000                  | 3500            |
| 45              | 1175            | 3600                 | 3075                  | 3750               | 4000             | 3150                  | 4200               | 3725                  | 3525            |
| 60              | 1300            | 3400                 | 3150                  | 3625               | 4025             | 2950                  | 4000               | 3000                  | 3525            |

15 The amounts of these materials to be employed will vary according to the composition of the rubber and the rubber mix and other conditions in a manner which will be readily apparent to one skilled in the art. For example, certain types of 18  
20 rubber may be more deficient in fatty acid than others and hence will require the use of larger amounts of material. Generally speaking, relatively small amounts are sufficient to produce the desired result and amounts of from 0.1 to 4.0% 25 will usually be found to be satisfactory in most cases.

It is also well known that certain accelerators, such as diphenyl guanidine are affected by the 30 presence of excessive amounts of free acid and in such cases the smallest amount of fatty acid which will overcome the fatty acid deficiency should be employed or the acids should be used in the form of their salts such as the zinc and lead salts. I have found that, when the acids of my invention 35 are employed, particularly in the form of metallic salts, they will not deleteriously affect the action of accelerators such as tetra-methyl-thiuram monosulfide, butyraldehyde-aniline condensation products and diphenyl guanidine.

40 While the acids and their salts are primarily intended to be employed in conjunction with organic accelerators, advantageous results may be obtained by employing these materials in the absence of added organic accelerator.

45 The acids of my invention and their metallic salts are sufficiently soluble in rubber so that effective amounts may be employed without the production of surface bloom or a non-tacky surface. Accordingly, these compounds are particularly 50 useful when a tacky surface is required to facilitate fabricating and building operations.

While I have disclosed the use of specific compounds within the class employed in specific proportions in only one rubber mix, it will be readily apparent to those skilled in the art that other

and they may be employed in other types of rubber mixes than that disclosed without departing from the spirit of my invention. Accordingly, the scope of my invention is to be limited solely by the appended claims, construed as broadly as is permissible in view of the prior art.

I claim:

1. The method of vulcanizing rubber which comprises incorporating in a rubber mix an organic accelerator of the type represented by mercaptobenzothiazole, diphenyl guanidine, tetra-methyl thiuram mono-sulfide and butyraldehyde-aniline and a small amount of an activator comprising a metal salt of propionic acid in which the metal is a member of the group consisting of zinc, lead, mercury and cadmium, and then subjecting the mix to a vulcanizing step.

2. The method of vulcanizing rubber which comprises incorporating in a rubber mix an organic accelerator of the type represented by mercaptobenzothiazole, diphenyl guanidine, tetra-methyl thiuram mono-sulfide and butyraldehyde-aniline and a small amount of an activator comprising zinc propionate, and then subjecting the mix to a vulcanizing step.

3. Rubber having incorporated therein an organic accelerator of the type represented by mercaptobenzothiazole, diphenyl guanidine, tetra-methyl thiuram mono-sulfide and butyraldehyde-aniline and a small amount of an activator comprising a metal salt of propionic acid in which the metal is a member of the group consisting of zinc, lead, mercury and cadmium.

4. Rubber having incorporated therein an organic accelerator of the type represented by mercaptobenzothiazole, diphenyl guanidine, tetra-methyl thiuram mono-sulfide and butyraldehyde-aniline and a small amount of an activator comprising zinc propionate.

IRA WILLIAMS. 55